

# United States Patent [19]

Kemp, Jr. et al.

[11] Patent Number: 4,780,131

[45] Date of Patent: \* Oct. 25, 1988

[54] **PROCESS FOR PRODUCING SPHERICAL LIGHT METAL BASED POWDER PARTICLES**

[75] Inventors: Preston B. Kemp, Jr., Athens; Walter A. Johnson, Towanda, both of Pa.

[73] Assignee: GTE Products Corporation, Stamford, Conn.

[\*] Notice: The portion of the term of this patent subsequent to Dec. 8, 2004 has been disclaimed.

[21] Appl. No.: 904,318

[22] Filed: Sep. 8, 1986

[51] Int. Cl.<sup>4</sup> ..... B22F 1/00

[52] U.S. Cl. ..... 75/0.5 B; 219/121.36; 264/15

[58] **Field of Search** ..... 75/0.5 R, 0.5 B, 10.19, 75/10.20; 219/121 P, 121 PB, 121 PY; 264/15

[56] **References Cited**

U.S. PATENT DOCUMENTS

3,974,245 8/1976 Chener et al. ..... 264/10  
4,264,354 4/1981 Cheetham ..... 75/0.5 B

4,711,660 12/1987 Kemp, Jr. ..... 75/0.5 B  
4,711,661 12/1987 Kemp, Jr. ..... 75/0.5 B

FOREIGN PATENT DOCUMENTS

02864 8/1984 European Pat. Off. ..... 75/0.5 B

*Primary Examiner*—Christopher W. Brody  
*Attorney, Agent, or Firm*—Donald R. Castle; L. Rita Quatrini

[57] **ABSTRACT**

A powdered material and a process for producing the material are disclosed. The powdered material consists essentially of light metal based spherical particles which are essentially free of elliptical shaped material and elongated particles having rounded ends. The process for making the spherical particles involves mechanically reducing the size of a starting material to produce a finer powder which is then entrained in a carrier gas and passed through a high temperature zone above the melting point of the finer powder to melt at least about 50% by weight of the powder and form spherical particles of the melted portion. The powder is directly solidified.

7 Claims, No Drawings

**PROCESS FOR PRODUCING SPHERICAL LIGHT METAL BASED POWDER PARTICLES**

**CROSS REFERENCE TO RELATED APPLICATIONS**

This invention is related to the following applications: Ser. No. 904,316, entitled "Fine Spherical Particles and Process For Producing Same," Ser. No. 905,015, entitled "Iron Group based And Chromium Based Fine Spherical Particles And Process For Producing Same," Ser. No. 904,997 entitled, "Spherical Refractory metal Based Powder Particles and Process For Producing Same", Ser. No. 905,011, now U.S. Pat. No. 4,711,661, entitled "Spherical Copper Based Powder Particles and Process For Producing Same," Ser. No. 905,013, now U.S. Pat. No. 4,711,660 entitled "Spherical Precious Metal Based Powder Particles and Process For Producing Same", and Ser. No. 904,317, entitled "Spherical Titanium Based Powder Particles And Process For Producing Same," all of which are filed concurrently herewith and all of which are by the same inventors and assigned to the same assignee as the present application.

**BACKGROUND OF THE INVENTION**

This invention relates to spherical powder particles and to the process for producing the particles which involves mechanically reducing the size of a starting material followed by high temperature processing to produce fine spherical particles. More particularly the high temperature process is a plasma process.

U.S. Pat. No. 3,909,241 to Cheney et al relates to free flowing powders which are produced by feeding agglomerates through a high temperature plasma reactor to cause at least partial melting of the particles and collecting the particles in a cooling chamber containing a protective gaseous atmosphere where the particles are solidified.

The only commercial process for producing fine spherical particles of light metals such as aluminum magnesium, and beryllium is by gas atomization. In some instances the process does not produce a high yield of spherical particles.

Therefore, a process for efficiently converting coarse, often non-spherical light metal based powder to spherical powder particles would be an advancement in the art.

In European Patent Application No. WO8402864 published Aug. 2, 1984, there is disclosed a process for making ultra-fine powder by directed a stream of molten droplets at a repellent surface whereby the droplets are broken up and repelled and thereafter solidified as described therein. While there is a tendency for spherical particles to be formed after rebounding, it is stated that the molten portion may form elliptical shaped or elongated particles with rounded ends.

**SUMMARY OF THE INVENTION**

In accordance with one aspect of this invention, there is provided a powdered material which consists essentially of light metal based spherical particles which are essentially free of elliptical shaped material and elongated particles having rounded ends.

In accordance with another aspect of this invention, there is provided a process for producing the above described spherical particles. The process for making the spherical particles involves mechanically reducing

the size of a starting material to produce a finer powder which is then entrained in a carrier gas and passed through a high temperature zone above the melting point of the finer powder to melt at least about 50% by weight of the powder and form spherical particles of the melted portion. The powder is directly solidified.

**DETAILED DESCRIPTION OF THE INVENTION**

For a better understanding of the present invention, together with other and further objects, advantages and capabilities thereof, reference is made to the following disclosure and appended claims in connection with the above description of some of the aspects of the invention.

The starting material of this invention is a light metal based material. The light metals on which the materials are based are aluminum, magnesium, and beryllium. The term "based materials" as used in this invention means any of the above described metals, or any of their alloys, with either of these possibly containing additives selected from the group consisting of oxides, nitrides, borides, carbides, silicides, as well as complex compounds such as carbonitrides, and mixtures thereof. One preferred light metal based material is aluminum with titanium diboride.

The size of the starting material is first mechanically reduced to produce a finer powder material. The starting material can be of any size or diameter initially, since one of the objects of this invention is to reduce the diameter size of the material from the initial size. Preferably the size of the major portion of the material is reduced to less than about 50 micrometers, with less than about 20 micrometers being preferred.

The mechanical size reduction can be accomplished by techniques such as by crushing, jet milling, attritor, rotary, or vibratory milling with attritor ball milling being the preferred technique for materials having a starting size of less than about 1000 micrometers in size.

A preferred attritor mill is manufactured by Union Process under the trade name of "The Szegvari Attritor". This mill is a stirred media ball mill. It is comprised of a water jacketed stationary cylindrical tank filled with small ball type milling media and a stirrer which consists of a vertical shaft with horizontal bars. As the stirrer rotates, balls impact and shear against one another. If metal powder is introduced into the mill, energy is transferred through impact and shear from the media to the powder particles, causing cold work and fracture fragmentation of the powder particles. This leads to particle size reduction. The milling process may be either wet or dry, with wet milling being the preferred technique. During the milling operation the powder can be sampled and the particle size measured. When the desired particle size is attained the milling operation is considered to be complete.

The particle size measurement throughout this invention is done by conventional methods as sedigraph, micromerograph, and microtrac with micromerograph being the preferred method.

The resulting reduced size material or finer powder is then dried if it has been wet such as by a wet milling technique.

If necessary, the reduced size material is exposed to high temperature and controlled environment to remove carbon and oxygen, etc.

The reduced size material is then entrained in a carrier gas such as argon and passed through a high temperature zone at a temperature above the melting point of the finer powder for a sufficient time to melt at least about 50% by weight of the finer powder and form essentially fine particles of the melted portion. Some additional particles can be partially melted or melted on the surface and these can be spherical particles in addition to the melted portion. The preferred high temperature zone is a plasma.

Details of the principles and operation of plasma reactors are well known. The plasma has a high temperature zone, but in cross section the temperature can vary typically from about 5500° C. to about 17,000° C. The outer edges are at low temperatures and the inner part is at a higher temperature. The retention time depends upon where the particles entrained in the carrier gas are injected into the nozzle of the plasma gun. Thus, if the particles are injected into the outer edge, the retention time must be longer, and if they are injected into the inner portion, the retention time is shorter. The residence time in the plasma flame can be controlled by choosing the point at which the particles are injected into the plasma. Residence time in the plasma is a function of the physical properties of the plasma gas and the powder material itself for a given set of plasma operating conditions and powder particles. Larger particles are more easily injected into the plasma while smaller particles tend to remain at the outer edge of the plasma jet or are deflected away from the plasma jet.

After the material passes through the plasma and cools, it is rapidly solidified. Generally the major weight portion of the material is converted to spherical particles. Generally greater than about 75% and most typically greater than about 85% of the material is converted to spherical particles by the high temperature treatment. Nearly 100% conversion to spherical particles can be attained. It is preferred that the major portion of the material have a particle size of less than about 50 micrometers with less than about 20 micrometers being especially preferred. The particle size of the plasma treated particles is largely dependent on the size of the material obtained in the mechanical size reduction step. As much as about 100% of the spherical particles can be less than about 50 micrometers.

The spherical particles of the present invention are different from those of the gas atomization process because the latter have caps on the particles whereas those of the present invention do not have such caps. Caps are the result of particle-particle collision in the molten or semi-molten state during the gas atomization event.

After cooling and resolidification, the resulting high temperature treated material can be classified to remove the major spheroidized particle portion from the essentially non-spheroidized minor portion of particles and to obtain the desired particle size. The classification can be done by standard techniques such as screening or air classification. The unmelted minor portion can then be reprocessed according to the invention to convert it to fine spherical particles.

The powdered materials of this invention are essentially relatively uniform spherical particles which are essentially free of elliptical shaped material and essentially free of elongated particles having rounded ends.

These characteristics can be present in the particles made by the process described in European Patent Application No. WO8402864 as previously mentioned.

Spherical particles have an advantage over non-spherical particles in injection molding and pressing and sintering operations. The lower surface area of spherical particles as opposed to non-spherical particles of comparable size, and the flowability of spherical particles makes spherical particles easier to mix with binders and easier to dewax.

A preferred powder of this invention is aluminum with titanium diboride.

Many of the light metals are consolidated into shapes by cold pressing followed by hot isostatic pressing. The powders of this invention enable more uniform consistent die filling by virtue of their spherical shape.

While there has been shown and described what are at present considered the preferred embodiments of the invention, it will be obvious to those skilled in the art that various changes and modifications may be made therein without departing from the scope of the invention as defined by the appended claims.

What is claimed is:

1. A process comprising:

(a) mechanically reducing the size of a light metal based material to produce a finer powder;

(b) entraining said finer powder in a carrier gas and passing said powder through a high temperature zone at a temperature above the melting point of said finer powder, said temperature being from about 5500° C. to about 17,000° C., said temperature being created by a plasma jet, to melt at least about 50% by weight of said finer powder to form essentially spherical particles of said melted portion; and

(c) rapidly and directly resolidifying the resulting high temperature treated material, while said material is in flight, to form spherical particles, said particles being essentially free of elliptical shaped material and essentially free of elongated particles having rounded ends.

2. A process of claim 1 wherein the size of said material is reduced by attritor milling to produce said finer powder.

3. A process of claim 1 wherein after said resolidification, said high temperature treated material is classified to obtain the desired particle size of said spherical particles.

4. A process of claim 1 wherein said light metal based material is a metal selected from the group consisting of aluminum, magnesium, and beryllium.

5. A process of claim 1 wherein said light metal based material is an alloy selected from the group consisting of aluminum alloys, magnesium alloys, and beryllium alloys.

6. A process of claim 1 wherein said light metal based material is a light metal with additives selected from the group consisting of oxides, nitrides, borides, carbides, silicides, carbonitrides, and mixtures thereof.

7. A process of claim 1 wherein said light metal based material is a light metal alloy with additives selected from the group consisting of oxides, nitrides, borides, carbides, silicides, carbonitrides, and mixtures thereof.

\* \* \* \* \*